

## UNITED STATES PATENT OFFICE

2,428,992

## MANUFACTURE OF SILICON MATERIAL FOR CRYSTAL CONTACTS

Charles Eric Ransley, Sudbury, John Walter Ryde, London W. 14, and Stanley Vaughan Williams, Kenton, England, assignors to The General Electric Company Limited, London, England

No Drawing. Application December 10, 1942, Serial No. 468,577. In Great Britain December 19, 1941

7 Claims. (Cl. 250—31)

1

This invention relates to the manufacture of silicon material for crystal contacts, suitable for use as electric rectifiers and mixers.

It has been proposed in patent application Serial No. 454,290 filed August 10, 1942, Patent Number 2,419,561 dated April 29, 1947, to introduce into the silicon a small quantity (e. g. not more than 2%) of aluminium and beryllium or a mixture of the two. If this additive is added to molten silicon and the melt is cooled slowly, it is sometimes found that the additive is not distributed uniformly in the solid material. When the material is broken up so as to yield the small pieces suitable for crystal contacts, some of these pieces may be almost free from additive, and therefore relatively unsuitable. This is the more likely to happen, the larger the amount of the melt. The object of this invention is to produce material in which the additive is consistently distributed with greater uniformity.

The probable explanation of the lack of uniformity is that the additive has a very low solubility in silicon at atmospheric temperature and therefore segregates during cooling, the segregation being the more complete the slower the cooling. Since the silicon is usually melted in vacuo, it is not convenient to quench the melt.

According to the invention, a process of manufacturing semi-conducting material for crystal contacts, comprising the step of melting silicon together with a small amount of additive, for example aluminium or beryllium or a mixture of aluminium and beryllium, and cooling the melt slowly to produce a solid product, comprises the further step, performed before the solid product is divided into pieces each suitable for a single contact, of maintaining the solid product for a considerable time at a temperature greatly above atmospheric temperature, but below the melting point of the product, and then quenching the product rapidly, the time and temperature of this heat treatment being chosen so that the additive is distributed approximately uniformly in the quenched product. In the said further step the product may be heated in air, but of course a neutral or reducing atmosphere may be used if it is desirable for any reason; the choice of atmosphere will only affect an outer skin of the product. The term "cool slowly" in the foregoing statement is correlative to the term "quench rapidly"; it implies that the rate of cooling during the "slow cooling" is much less than in the "rapid quenching."

On theoretical grounds it is probable that the minimum temperature at which the heat treat-

2

ment will produce the desired result is that at which the additive is completely soluble in the silicon. Since the solubility is a maximum at the eutectic temperature, the said minimum temperature cannot be higher than the eutectic temperature, which is about 575° C. for aluminium and 1090° C. for beryllium. The eutectic temperature of the system aluminium-beryllium-silicon appears not to be known. We have found that, when the additive is 1/4% of aluminium, heating at 575°-580° C. for several hours will produce the desired result. But if the amount of the additive is less than that corresponding to the eutectic (which will certainly be the case when the additive is beryllium), the minimum temperature may be much below the eutectic temperature; moreover there is no reason why temperatures approaching the minimum should be used. Accordingly these theoretical considerations are of little value as a guide to practice. Whether the additive is aluminium or beryllium or a mixture of the two (we have found 1/4% aluminium and 1/2% beryllium very suitable), maintaining the product at 1050° C. for one hour and then quenching in water has been found to produce the desired uniformity; we know of no reason why any other heat treatment should be used.

In the said application Serial No. 454,290 it was proposed that the additive should be added in the form of metal mixed with the silicon before the melt. However the additive, especially when it is or contains beryllium, may be introduced into the silicon partly or wholly by reaction of the silicon during the melting with the material of the crucible in which the melting takes place. The method by which the additive is introduced into the melt is irrelevant to the invention; and we desire it to be understood that in the foregoing statement of the invention and in the appended claims, the phrase "melting silicon together with a small amount of additive" is to be interpreted to include any step in which a mixture of silicon and the additive is maintained for an appreciable time in the molten state.

We claim:

1. A process of manufacturing semi-conducting material for crystal contacts, comprising the step of melting silicon together with a small amount of additive, and cooling the melt slowly to produce a solid product, which comprises the further step, performed before the solid product is divided into pieces each suitable for a single contact, of maintaining the solid product for a considerable time at a temperature greatly above atmospheric temperature, but below the melting

## 3

point of the product, and then quenching the product rapidly, the time and temperature of this heat treatment being chosen so that the additive is distributed approximately uniformly in the quenched product.

2. A process of manufacturing semi-conducting material for crystal contacts, comprising the step of melting silicon together with a small amount of aluminium, and cooling the melt slowly to produce a solid product, which comprises the further step, performed before the solid product is divided into pieces each suitable for a single contact, of maintaining the solid product for a considerable time at a temperature greatly above atmospheric temperature, but below the melting point of the product, and then quenching the product rapidly, the time and temperature of this heat treatment being chosen so that the aluminium is distributed approximately uniformly in the quenched product.

3. A process of manufacturing semi-conducting material for crystal contacts, comprising the step of melting silicon together with a small amount of beryllium, and cooling the melt slowly to produce a solid product, which comprises the further step, performed before the solid product is divided into pieces each suitable for a single contact, of maintaining the solid product for a considerable time at a temperature greatly above atmospheric temperature, but below the melting point of the product, and then quenching the product rapidly, the time and temperature of this heat treatment being chosen so that the beryllium is distributed approximately uniformly in the quenched product.

4. A process of manufacturing semi-conducting material for crystal contacts, comprising the step of melting silicon together with a small amount of a mixture of aluminium and beryllium, and cooling the melt slowly to produce a solid product, which comprises the further step, performed before the solid product is divided into pieces each suitable for a single contact, of main-

## 4

taining the solid product for a considerable time at a temperature greatly above atmospheric temperature, but below the melting point of the product, and then quenching the product rapidly, the time and temperature of this heat treatment being chosen so that the mixture of aluminium and beryllium is distributed approximately uniformly in the quenched product.

5. A process of manufacturing semi-conducting material for crystal contacts, comprising the step of melting silicon together with a small amount of aluminium, and cooling the melt slowly to produce a solid product, which comprises the further step, performed before the solid product is divided into pieces each suitable for a single contact, of maintaining the solid product for one hour at a temperature of 1050° C. and then quenching the product rapidly.

6. A process of manufacturing semi-conducting material for crystal contacts, comprising the step of melting silicon together with a small amount of beryllium, and cooling the melt slowly to produce a solid product, which comprises the further step, performed before the solid product is divided into pieces each suitable for a single contact, of maintaining the solid product for one hour at a temperature of 1050° C. and then quenching the product rapidly.

7. A process of manufacturing semi-conducting material for crystal contacts, comprising the step of melting silicon together with a small amount of a mixture of aluminium and beryllium, and cooling the melt slowly to produce a solid product, which comprises the further step, performed before the solid product is divided into pieces each suitable for a single contact, of maintaining the solid product for one hour at a temperature of 1050° C. and then quenching the product rapidly.

40

CHARLES ERIC RANSLEY.

JOHN WALTER RYDE.

STANLEY VAUGHAN WILLIAMS.